

[54] LIGHT-SENSITIVE SILVER HALIDE  
COLOR-PHOTOGRAPHIC EMULSIONS[72] Inventors: **Masakuni Iwama; Isaburo Inoue; Teruo Hanzawa; Kenro Sakamoto; Takaya Endo**, all of Tokyo, Japan[73] Assignee: **Konishiroku Photo Industry Co., Ltd.**, Chuo-ku, Tokyo, Japan[22] Filed: **Aug. 6, 1969**[21] Appl. No.: **848,069**

## [30] Foreign Application Priority Data

Aug. 12, 1968 Japan.....43/56727

[52] U.S. Cl.....96/100, 250/65

[51] Int. Cl.....G03c 1/40

[58] Field of Search.....96/100, 9

## [56] References Cited

## UNITED STATES PATENTS

2,652,329 9/1953 McCrossen et al. ....96/100

3,135,609 6/1964 Klinger .....96/100  
3,468,665 9/1969 Misu et al. ....96/100Primary Examiner—J. Travis Brown  
Attorney—Waters, Roditi, Schwartz & Nissen

## [57] ABSTRACT

A light-sensitive silver halide color-photographic emulsion which contains as protected coupler, a compound of the general formula



wherein B is a coupler residue;

 $nR_1$  are hydrogen atoms, or at most one of  $nR_1$  is a  $C_1$  to  $C_{18}$ -aliphatic hydrocarbon radical, attached to the terminal carbon of the alkylene chain and the remaining  $(n-1)R_1$  are hydrogen; $R_2$  is a  $C_7$  to  $C_{18}$ -aliphatic hydrocarbon radical;

X is a group capable of bonding the coupler residue with an acylamino group;

 $n$  is 2 or 3; and $q$  is 1 or 2.

8 Claims, No Drawings

LIGHT-SENSITIVE SILVER HALIDE COLOR-  
PHOTOGRAPHIC EMULSIONS

This invention relates to a light-sensitive color-photographic emulsion. More particularly, it relates to a light-sensitive silver halide color-photographic emulsion which comprises, as a protected coupler, a new compound of the general formula



wherein B is a coupler residue;  $nR_1$  are hydrogen atoms, or at most one of the  $nR_1$  is a  $C_1$  to  $C_4$  — aliphatic hydrocarbon radical attached to the terminal carbon atom of the alkylene chain and the remaining  $(n-1)R_1$  are hydrogen atoms;  $R_2$  is a  $C_7$  to  $C_{18}$  — aliphatic hydrocarbon radical, X is a group being capable of bonding the coupler residue with an acylamino group,  $n$  is 2 or 3 and  $q$  is 1 or 2.

Various compounds have been proposed as protected couplers heretofore. However, they usually suffer from individual disadvantages. Few protected coupler compounds are known which can be prepared at an inexpensive cost and in high purity.

For example, a coupler compound of the formula



is disclosed in U.S. Pat. No. 2,801,171. Although this compound advantageously has good solubility in high boiling solvents, it must be prepared from a very expensive starting material and is difficult to purify.

Another coupler of the formula



is disclosed in Japanese Pat. Publn. No. 2835/1964. It also has good solubility in high boiling solvents. However, it is quite expensive because its oleophilic portion must be prepared through several steps from an expensive starting material.

In view of the above-mentioned disadvantages of the prior art, it is one object of the invention to provide a light-sensitive color-photographic emulsion which contains a coupler compound, with superior photographic characteristics to those of conventionally known coupler compounds. Another object of the invention is to provide a light-sensitive color-photographic emulsion which when coated can form a stable light-sensitive color-photographic film free from crystallization of the coupler contained therein. Still another object of the invention is to provide a new coupler compound which can be obtained at an economical cost and in high purity.

Coupler compounds usable in the present invention have the following advantages:

1. They can be prepared by a simple and economical way starting from a long-chain alcohol easily available in the market,
2. they have good solubilities in dibutyl phthalate, tricresyl phosphate or the like high boiling solvents, so that a highly concentrated, stable coupler dispersion is obtainable because of the possibility of reducing solvent amounts required for couplers, and
3. they are unlikely to crystallize from the emulsion or coating containing same, because of their low melting point.

These couplers are very useful as protected couplers in the art of color photography and can be synthesized in the following way.

A long-chain alcohol and a dibasic carboxylic acid anhydride (e.g., succinic anhydride or glutaric anhydride) are brought into reaction to form a dibasic carboxylic acid monoalkyl ester, which is then reacted with thionyl chloride. The acid chloride thus obtained is condensed with a coupler component having an amino group thereby obtaining the desired coupler compound. The above process can be represented by the following chemical formulas.



In the above formulas,  $R_1$ ,  $R_2$ , B, X,  $n$  and  $q$  have the same meanings as defined above, and  $p$  is 1 or 2.

In the general formula of the coupler compounds of the invention, the coupler residue (B) is a residue of a phenolic hydroxy-bearing compound (e.g., phenol, naphthol, etc.) or a derivative thereof or of an active methylene-bearing compound (e.g., pyrazolone, indazolone, acylacetanilide, etc.) or a derivative thereof. Further, the group X may be any group capable of bonding the coupler residue with an acylamino group and it includes, for example, an imino group or a residue of an imino-bearing alkylene or arylene derivative.

Typical compounds of the couplers of the present invention are listed below, without limiting the scope of the invention thereto.







Typical synthetic procedures for these couplers will be mentioned below.

Synthesis Example (1)

105 g. of succinic anhydride is heated on an oil bath. To the resulting melt, 187 g. of n-dodecyl alcohol is added, and the mixture is stirred at 120°-125° C. for 3 hours. After cooling, the solidified mass is recrystallized from hexane. Succinic acid mono-n-dodecyl ester melting at 44.5°-45.5° C. is obtained. 143 g. of this ester is mixed with 140 g. of thionyl chloride and the mixture is allowed to stand overnight. The thionyl chloride is removed by distillation under reduced pressure. The remaining mass, succinic acid mono-n-dodecyl ester chloride, is passed to the next acylation.

To the mixture of 500 ml. of glacial acetic acid and 9.0 g. of anhydrous sodium acetate, 28.0 g. of  $\alpha$ -(3-aminobenzoyl)-2-methoxy-acetanilide and 40.0 g. of the above-resulted chloride are added. The mixture is heated on a water bath for 2 hours and then poured into water. The precipitate formed is collected by filtration, washed with water and then dried. The crude product is recrystallized from a mixed solvent of benzene and hexane thereby to obtain the coupler (1), indicated before, as a white powder melting at 103°-104° C. Yield 40.0 g. (74 percent on theoretical basis). The elemental analysis shows the following.

N  
Calcd. : 5.07%  
Found : 4.78%

By repeating the above procedures in the substantially same manner, the couplers (2), (3) and (4) can be obtained.

| Coupler | m.p. (°C.) | Nitrogen analysis (%) |       |
|---------|------------|-----------------------|-------|
|         |            | Calcd.                | Found |
| No. (2) | 92-93      | 5.22                  | 5.32  |
| No. (3) | Oil        | 4.77                  | 5.25  |
| No. (4) | 61-62      | 4.59                  | 4.80  |

Synthesis Example (2)

39.8 g. of 1-(2,4,6-trichlorophenyl)-3-(3-aminobenzamido)-5-pyrazolone is suspended in the mixture of 200 ml. of acetonitrile and 40 ml. of pyridine, 42.0 g. of succinic acid mono-n-dodecyl ester chloride is added to the suspension, which is then boiled for 1 hour. Then, this suspension is added with water and the separated oil is extracted with ethyl acetate. The extract is washed with water, dried and then freed from the solvent. The remaining oil is dissolved in methyl alcohol and the resulting solution is passed through ion-exchange columns individually packed with Amberlite CG 120 and Amberlite CG 400 of Rohm & Haas Co., U.S.A. Solvent is removed from the treated solution by distillation and the remaining mass is recrystallized from a mixed solvent of benzene and hexane. A pale yellow powder melting at 77°-78° C. is obtained. This is the coupler (6), indicated before, Yield 39 g. (59 percent on theoretical basis).

By repeating the above procedures in substantially the same

manner, the couplers (5) to (11) and (15) to (16), indicated before, are obtained.

| 5        | Coupler | m.p. (°C.) | Nitrogen analysis (%) |       |
|----------|---------|------------|-----------------------|-------|
|          |         |            | Calcd.                | Found |
| No. (5)  |         | 51-52      | 8.30                  | 8.15  |
| No. (6)  |         | 77-78      | 8.41                  | 8.17  |
| No. (7)  |         | 85-87      | 8.96                  | 8.70  |
| No. (8)  |         | 132-133    | 8.33                  | 8.20  |
| No. (9)  |         | 65-68      | 9.16                  | 8.92  |
| No. (10) |         | 182-183    | 8.83                  | 9.09  |
| No. (11) |         | 156-157    | 7.88                  | 7.86  |
| No. (15) |         | 61-64      | 3.37                  | 3.34  |
| No. (16) |         | 152-155    | 4.27                  | 4.29  |

Synthesis Example (3)

15 22.9 g. of 2-amino-4,6-dichloro-5-methyl-phenol hydrochloride is mixed with 550 ml. of acetone and 25.0 g. of diethyl aniline. The resulting mixture is added with 40.0 g. of succinic acid mono-n-dodecyl ester chloride and then stirred for 1 hour, followed by boiling for 1 hour. The reaction mixture is filtered, and the filtrate is concentrated and then the remaining oil is added to a mixture of conc. HCl and water. The solidified oily mass is collected by filtration, washed with water, dried and then recrystallized from acetonitrile thereby 20 obtaining 30.0 g. (yield 65 percent) of a white powder melting at 72°-74° C. The product is the coupler (14). The nitrogen analysis shows the following.

N  
30 Calcd. : 3.04%  
Found : 3.19%

Synthesis Example (4)

35 3.6 g. of p-anisidine, 40.0 ml. of water, 10.0 ml. of concentrated hydrochloric acid and 2.4 g. of sodium nitrite are brought into reaction, followed by addition of 80 ml. of ethyl alcohol.

The diazotized solution thus prepared is added at 5°-10° C. to a solution of 12.8 g. of the coupler (8) in 128 ml. of 40 pyridine. The resulting mixture is stirred for 3 hours and then diluted with 300 ml. of water; 128 ml. of concentrated hydrochloric acid is added thereto, and the separated precipitate is collected by filtration, washed with water, dried and then recrystallized from ligroin thereby to obtain 11.6 g. 45 (yield 85 percent) of orange powder melting at 106°-107° C. This product is the coupler (13), indicated before.

By repeating the above procedures in the same manner as above, but using 1-(2,4,6-trichlorophenyl)-3-[4-( $\beta$ -dodecyloxy-carbonylethyl-carbamyl)-anilino]-5-pyrazolone 50 instead of the coupler (8), the coupler (12) can be obtained.

Further by repeating the above procedures in the same manner as above but using the diazotized 0-amino-acetophenone and the coupler (15) instead of the diazotized p-anisidine and the coupler (8) respectively, the coupler (17) 55 can be obtained.

The melting points and nitrogen analyses of these couplers are shown below.

| 60       | Coupler | m.p. (°C.) | Nitrogen analysis (%) |       |
|----------|---------|------------|-----------------------|-------|
|          |         |            | Calcd.                | Found |
| No. (13) |         | 106-107    | 10.42                 | 10.26 |
| No. (12) |         | 85-87      | 10.88                 | 10.70 |
| No. (17) |         | 126-127    | 9.68                  | 9.41  |

65 In order to prepare a light-sensitive color-photographic emulsion of the invention, any one of the couplers prepared as above is dissolved in a high boiling solvent (b.p. 175° C. or higher) such as tricresyl phosphate, dibutyl phthalate, etc. or a low boiling solvent such as butyl acetate, butyl propionate, etc. or a mixture of both. The thus prepared solution may be 70 mixed with an aqueous gelatinous solution containing a surface active agent.

Then, the coupler dispersion thus obtained is emulsified by means of a high speed rotary mixer or colloid mill and then added directly to a light-sensitive silver halide photographic emulsion, which is coated on a suitable support (e.g., film

base, baryta paper, etc.), followed by drying to remove the majority of the low boiling solvent. Alternatively, the emulsified coupler dispersion is set and extruded to noodle form, followed by water-washing or the like procedure to remove the low boiling solvent. Then it is added to a light-sensitive silver halide photographic emulsion, which in turn is coated on a support and dried to obtain a light-sensitive silver halide photographic material. It should be understood that the manner of incorporation of the couplers into a light-sensitive photographic emulsion as mentioned above is merely illustrative and does not limit the scope of the invention in any way.

The preferred amount of the coupler in photographic emulsion usually is 10-100 g. per mole of silver halide. However, this is not critical and can be varied depending on the purpose of the final use. The light-sensitive silver halide emulsion may contain any type of silver salts including silver chloride, silver iodide or silver chloroiodide. Further, said emulsion may contain any sensitizer, for example, sulfur sensitizer, polyalkylene oxide sensitizer, noble metal sensitizer, etc. Other photographic additives may exist in the photographic emulsion, which are antifoggants, stabilizers, anti-stain agents, anti-irradiation agents, coating aids, etc. Known optical sensitizers,

e.g., cyanine dyes, merocyanine dyes, etc., also may be contained therein.

A light-sensitive silver halide color-photographic material obtained from the above-mentioned light-sensitive silver halide color-photographic emulsion can be subjected to exposure by actinic irradiation ( $\alpha$ -ray,  $\beta$ -ray, X-ray, visible ray, infrared ray, etc.) and then treated with a liquid developer containing a p-phenylene diamine type compound. The resulting developed image is bleached and fixed, thereby giving a highly transparent color image having good spectral absorption characteristics.

Typical p-phenylene diamine type compounds which are contained as the main active ingredient in the liquid developer are the sulfates, sulfites and hydrochlorides of N,N-diethyl-p-phenylene diamine, N-ethyl-N- $\beta$ -methane-sulfonamidoethyl-3-methyl-4-aminoaniline, N-ethyl-N-hydroxyethyl-p-phenylene diamine, N-ethyl-N-hydroxyethyl-2-methyl-p-phenylene diamine, N,N-diethyl-2-methyl-p-phenylene diamine and the like.

The melting points of the couplers of the present invention are compared with those of known couplers having a similar structure in Table 1.

TABLE 1

| Coupler                          | Structure | M.p. (° C.) |
|----------------------------------|-----------|-------------|
| Coupler (1).....                 |           | 103-104     |
| Coupler of U.S.P. 2,875,057..... |           | 126-127     |
| Coupler (6).....                 |           | 77-78       |
| Coupler of U.S.P. 2,618,641..... |           | 138-139     |
| Coupler (14).....                |           | 72-74       |
| Coupler of U.S.P. 2,801,171..... |           | 123-124     |

The above data clearly indicate that the couplers of the present invention have remarkably lower melting points than the conventionally known couplers.

Further, some test results demonstrating the high solubility of the couplers of the present invention in high boiling solvents are shown in Table 2. Degree of solubility is expressed in terms of the dibutyl phthalate amount (ml.) required for dissolution of 1.0 g. of the particular coupler at 60°C.

## EXAMPLE 1

20 g. of the coupler (1), indicated before, is dissolved at 60°C. in the mixture of 20 ml. of dibutyl phthalate and 60 ml. of butyl acetate. The resulting clear solution is mixed with 10 ml. of an aqueous solution of 10 percent Alkanol B (alkyl naphthalene sulfonate, manufactured and sold by Du Pont, U.S.A.) and 200 ml. of an aqueous solution of 5 percent

TABLE 2

| Coupler                          | Structure | Dibutyl phthalate amount (ml.) |
|----------------------------------|-----------|--------------------------------|
| Coupler (1).....                 |           | 5.0                            |
| Coupler of U.S.P. 2,875,057..... |           | 7.5                            |
| Coupler (6).....                 |           | 1.5                            |
| Coupler of U.S.P. 2,618,641..... |           | 2.0                            |
| Coupler (14).....                |           | 2.0                            |
| Coupler of U.S.P. 2,801,171..... |           | 3.0                            |

The above data clearly indicated that the couplers of the present invention are superior in solubility in high boiling solvents to the conventionally known couplers, and this affirms the usefulness of our couplers as protected couplers in color-photography.

Accordingly, it can be understood that a light-sensitive silver halide color-photographic emulsion of the invention which comprises a coupler of the above-defined general formula is quite free from crystallization of the coupler, with the result that said emulsion can give an excellent color image having good spectral absorption characteristics and good transparency, due to non-existence of irregular spectral absorption.

Now the following examples will serve to show the invention in detail, without limiting the scope of the invention thereto.

gelatine. The mixture is treated by means of a colloid mill.

The thus prepared coupler dispersion is added to 1 kg. of a high speed gelatino silver iodobromide emulsion, which in turn is coated on a film base and dried. A light-sensitive photographic film having a stable light-sensitive layer is obtained.

This photographic film is exposed to light in the usual manner and then treated at 20°C. for 10 minutes with a liquid developer of the following formulation:

|    |                                               |         |
|----|-----------------------------------------------|---------|
| 70 | N,N-diethyl-p-phenylene diamine hydrochloride | 2.5 g.  |
|    | Anhydrous sodium sulfite                      | 2.0 g.  |
|    | Sodium carbonate monohydrate                  | 82.0 g. |
|    | Potassium bromide                             | 2.0 g.  |
|    | Water to make up 1,000 ml.                    |         |

The treated film is then treated with a stopping solution and a fixing solution, washed with water for 10-15 minutes and then treated for 5 minutes with a bleaching solution of the following formulation:

|                            |        |
|----------------------------|--------|
| Potassium ferricyanide     | 100 g. |
| Potassium bromide          | 50 g.  |
| Water to make up 1,000 ml. |        |

The film is washed with water for 5 minutes and then treated for 5 minutes with a fixing solution of 250 g. of sodium thiosulfate in 1,000 ml. of water. Washing with water for 20-25 minutes is made, followed by drying. A brilliant yellow color image having absorption maximum at 440 m $\mu$  is obtained.

Substantially the same procedures as above are repeated but using the coupler (6) or coupler (15) instead of the coupler (1). A clear magenta or cyan color image having an absorption maximum at 540 m $\mu$  or 670 m $\mu$ , respectively, can be obtained.

#### EXAMPLE 2

10 g. of the coupler (2), indicated before, is dissolved at 50° C. in 10 ml. of tricresyl phosphate and 30 ml. of butyl acetate. The resulting clear solution is mixed with 5 ml. of an aqueous solution of 10 percent Alkanol B and 800 ml. of an aqueous solution of 5 percent gelatine. The resulting mixture is treated in a colloid mill.

The coupler dispersion thus obtained is added to 500 g. of a light-sensitive gelatino silver iodobromide emulsion, which in turn is coated on a film base and dried.

The light-sensitive silver halide photographic film thus obtained is exposed to light and then treated at 20° C. for 10 minutes with a liquid developer of the following formulation:

|                            |         |
|----------------------------|---------|
| Methol                     | 3.0 g.  |
| Anhydrous sodium sulfite   | 60.0 g. |
| Hydroquinone               | 6.0 g.  |
| Anhydrous sodium carbonate | 50.0 g. |
| Potassium bromide          | 1.0 g.  |
| Water to make up 1,000 ml. |         |

After stopping, film hardening and water-washing in the usual manner, the film is further subjected to secondary exposure to light and then treated at 20° C. for 10 minutes with a liquid developer of the following formulation:

|                                               |         |
|-----------------------------------------------|---------|
| N,N-diethyl-p-phenylene diamine hydrochloride | 5.0 g.  |
| Anhydrous sodium sulfite                      | 2.0 g.  |
| Sodium carbonate (monohydrate)                | 82.0 g. |
| Potassium bromide                             | 1.0 g.  |
| Water to make up 1,000 ml.                    |         |

The film is then treated by stopping, fixing, water-washing and bleaching in the usual manner and then washed with running water for 20 minutes and dried. A yellow color positive image having good transparency and having an absorption maximum at 445 m $\mu$  is obtained.

Substantially the same procedures as above are repeated but using the coupler (8) or (16) instead of the coupler (2). A clear magenta or cyan color image having an absorption maximum at 535 m $\mu$  or 680 m $\mu$ , respectively, can be obtained.

#### EXAMPLE 3

10 g. of the coupler (14), indicated before, is dissolved at 50° C. in 20 ml. of dibutyl phthalate. The resulting clear solution is mixed with 5 ml. of an aqueous 10 percent Alkanol B solution and 200 ml. of an aqueous 5 percent gelatine solution. The resulting mixture is passed several times through a colloid mill.

The coupler dispersion thus prepared is added to 500 g. of a light-sensitive gelatino silver chlorobromide emulsion, which in turn is coated on a baryta paper and dried.

The light-sensitive silver halide photographic film thus prepared, after light exposure, is treated at 20° C. for 10 minutes in a developing bath of the following formulation:

|    |                                                         |         |
|----|---------------------------------------------------------|---------|
| 5  | N-ethyl-N-hydroxyethyl-p-phenylenediamine hydrochloride | 2.5 g.  |
|    | Anhydrous sodium sulfite                                | 2.0 g.  |
|    | Hydroxylamine hydrochloride                             | 1.0 g.  |
|    | Sodium carbonate (monohydrate)                          | 82.0 g. |
| 10 | Potassium bromide                                       | 2.0 g.  |
|    | Water to make up 1,000 ml.                              |         |

The film is then immersed in a stopping bath consisting of 10 ml. of glacial acetic acid, 3.0 g. of sodium hydroxide and 1,000 ml. of water, and immediately thereafter, immersed in a film hardener-containing fixing bath for 4 minutes. After water-washing for 10 minutes, the film is treated at 20° C. for 8 minutes in a bleaching bath of the following formulation:

|    |                                                |        |
|----|------------------------------------------------|--------|
| 20 | Ethylenediamine tetraacetic acid disodium salt | 40 g.  |
|    | Ferric chloride                                | 30 g.  |
|    | Sodium carbonate (monohydrate)                 | 20 g.  |
|    | Potassium bromide                              | 30 g.  |
| 25 | Sodium thiosulfate                             | 200 g. |
|    | Water to make up 1,000 ml.                     |        |

After washing with water for 20 minutes, the film is immersed in a stabilizing bath for 2 minutes and then dried. A cyan color image having good light fastness and humidity resistance and having an absorption maximum at 680 m $\mu$  is obtained.

#### EXAMPLE 4

2.0 g. of the coupler (13), indicated before, is dissolved at 60° C. in 2 ml. of dibutyl phthalate and 6 ml. of butyl acetate. The resulting clear solution is mixed with 1 ml. of an aqueous 10 percent Alkanol B solution and 20 ml. of an aqueous 5 percent gelatine solution.

The coupler dispersion thus prepared is added to 100 g. of a high speed light-sensitive gelatino silver iodobromide photographic emulsion, which in turn is coated on a film base and dried.

After light-exposure in the usual manner, the light-sensitive photographic film is treated with a color developer as used in Example 1. A yellow color positive image having an absorption maximum at 440 m $\mu$  and a magenta color image having an absorption maximum at 540 m $\mu$  are obtained.

Substantially the same procedures as above are repeated but using the coupler (17) instead of the coupler (13). A red color positive image having an absorption maximum at 520 m $\mu$  and a cyan color image having an absorption maximum at 670 m $\mu$  are obtained.

#### EXAMPLE 5

5.0 g. of the coupler (15), indicated before, is dissolved at 60° C. in 5.0 ml. of dibutyl phthalate and 15 ml. of butyl acetate. The resulting clear solution is mixed with 2.5 ml. of an aqueous 10 percent Alkanol B solution and 50 ml. of an aqueous 5 percent gelatine solution. The mixture is treated by means of a colloid mill.

The coupler dispersion thus prepared is added to 500 g. of a light-sensitive silver chloride photographic emulsion sensitized at the wavelength region of red light. This emulsion in turn is coated on a film base and dried.

65 The light-sensitive photographic film thus prepared is exposed to X-ray irradiation in the usual manner and then treated at 20° C. for 10 minutes with a developer as used in Example 1. After stopping, film-hardening and water-washing in the usual manner, the treated film is subjected to secondary exposure to yellow light (exposure time 30 seconds, Agfa-reprocolor separation filter used) and then treated at 20° C. for 10 minutes with the same developer as above. Stopping, fixing, bleaching, water-washing and drying are carried out in the usual manner. A clear yellow color image on a blue background is obtained.

## EXAMPLE 6

5.0 g. of the coupler (6) is dissolved at 60° C. in the mixture of 5.0 ml. of dibutyl phthalate and 15 ml. of butyl acetate. The resulting clear solution is mixed with 2.5 ml. of an aqueous 10 percent Alkanol B solution and 50 ml. of an aqueous 5 percent gelatine solution. The resulting mixture is treated in a colloid mill.

The thus obtained coupler dispersion is added to 500 g. of a high speed light-sensitive silver iodobromide photographic emulsion, which in turn is coated on a film base and dried to obtain a light-sensitive silver halide photographic film.

Separately, a gelatine layer having a dry thickness of about 5  $\mu$  is prepared on a cellulose triacetate film. On that layer, a tritium-labelled thymidine solution is spotted at the ratio of 10  $\mu$ c. (micro-count) per square centimeters. Then, spotting is repeated by using double dilution of the said solution. By repeating this method, a standard tritium radiation source having a stepwedge of radioactivity in geometric progression with an equal ratio of 2 is prepared.

The gelatine layer of this radiation source is brought into contact with the light-sensitive layer of the light-sensitive photographic film and the resultant composite is allowed to stand for 15 hours in a dark room. At the end of that time, the gelatine layer is removed and the photographic film is treated by the developing procedures mentioned in Example 1. A magenta color image which indicates the existence of the radioactive substance is formed at the position which corresponds to the radioactive source of the gelatine layer.

What we claim is:

1. A light-sensitive silver halide color-photographic emulsion which contains, as protected coupler, a compound of the general formula



wherein B is a coupler residue;

$nR_1$  are hydrogen atoms, or at most one of  $nR_1$  is a  $C_1$  to  $C_4$  aliphatic hydrocarbon radical, attached to the terminal carbon of the alkylene chain and the remaining  $(n-1)R_1$  are hydrogen;

$R_2$  is a  $C_7$  to  $C_{18}$  aliphatic hydrocarbon radical;

X is a group capable of bonding the coupler residue with an acylamino group;

$n$  is 2 or 3; and

$q$  is 1 or 2.

2. A light-sensitive silver halide color-photographic emulsion as claimed in claim 1, wherein said protected coupler is a compound of the structural formula



3. A light-sensitive silver halide color-photographic emulsion as claimed in claim 1, wherein said protected coupler is a compound of the structural formula



4. A light-sensitive silver halide color-photographic emulsion as claimed in claim 1, wherein said protected coupler is a compound of the structural formula



5. A light-sensitive silver halide color-photographic emulsion as claimed in claim 1, wherein said protected coupler is a compound of the structural formula



6. A light-sensitive silver halide color-photographic emulsion as claimed in claim 1, wherein said protected coupler is a compound of the structural formula



45

7. A light-sensitive silver halide color-photographic emulsion as claimed in claim 1, wherein said protected coupler is a compound of the structural formula



8. A light-sensitive silver halide color-photographic emulsion as claimed in claim 1, wherein said protected coupler is a compound of the structural formula

